

1

2,797,161

## MAGNET ALLOY

James R. Ireland and Stephen Lester, Indianapolis, Ind., assignors to Thomas & Skinner, Inc., a corporation of Indiana

No Drawing. Application September 3, 1953,  
Serial No. 378,396

1 Claim. (Cl. 75—124)

This invention relates to improvements in magnet alloys of the type represented by the alloys known as Alnico V and Alnico VI.

In their general formula, the Alnico V and Alnico VI type magnet alloys contain from 6% to 11% aluminum, from 10% to 20% nickel, from 16% to 30% cobalt, and up to about 7% copper. High magnetic strength alloys of this general formula also contain small amounts of additive constituents, that is, up to about 1.0% manganese, and up to about 1.0% silicon. One of the highest-strength Alnico V alloys also contains a small percentage of zirconium. One of the highest-strength Alnico VI alloys contains, in addition, a small percentage of titanium. The balance, in each case, is substantially all iron.

It is an object of the invention to provide an improved magnet alloy having higher magnetic properties than have heretofore been obtained. It is an object of the invention to provide a magnet alloy having high magnetic properties in combination with desirable physical properties. It is an object of the invention to provide an alloy formula which will give magnets of the desired properties with a high degree of uniformity, and which will facilitate the regular commercial production of high-strength magnets of desirable physical properties. It is an object of the invention to provide a magnet alloy in which the presence of impurities, especially carbon, is less critical than has heretofore been the case.

In accordance with our invention, we include in the magnet alloy a small percentage of columbium, and preferably also a small percentage of sulphur. The columbium eliminates the need for zirconium, and we find that by the use of columbium instead of zirconium, we obtain improved results and provide an alloy of less cost than the known zirconium-containing alloys.

We find that the use of columbium, preferably also with sulphur, greatly improves the uniformity with which alloys of this type can be produced. We find, especially with Alnico V alloys, that the use of columbium produces a magnet alloy of substantially improved magnetic properties. While with columbium alone, the alloy tends to give magnets of poor physical properties, which may be so brittle that they crumble during production grinding operations, the addition of sulphur with the columbium avoids such poor physical properties and gives an alloy of improved magnetic properties combined with adequate physical toughness.

In accordance with our invention, the amount of columbium included in the alloy can be between 0.05% to 1.0%, and preferably between about 0.05% and 0.4%. The amount of sulphur used is desirably at least one quarter the amount of columbium used, and can be between 0.01% and 0.3%, and preferably between 0.02% and 0.1%.

Our new magnet alloy containing columbium and sulphur provides higher magnetic properties than have heretofore been obtained with Alnico V alloys. It permits those increased magnetic properties to be obtained uniformly on successive heats, and provides an alloy of adequate strength and toughness, so that there is a substantial reduction in the amount of material lost as scrap. In addition, like the addition of zirconium, our

2

use of columbium and sulphur permits a reduction in the percentage of cobalt and nickel from that required to obtain best results with the standard Alnico V alloy; and while columbium is itself more expensive than zirconium, the amount required is substantially less so that the cost of the added ingredient and of the over-all alloy is less than when zirconium is used. Further, we find that the use of columbium and sulphur permits the obtaining of good results even when carbon is present to a relatively high degree, say up to about 0.05%, so that there is a less critical necessity for extreme reductions in the amount of carbon present. Our new alloy does not require the presence of manganese, but a small percentage of manganese may be present.

15 The following Table 1 shows in column I the preferred range of constituents for alloys embodying our invention, and in column II a range which we have found to be most desirable:

TABLE 1

|    | Constituents         | I<br>Preferred<br>Range,<br>percent | II<br>Optimum<br>Range,<br>percent |
|----|----------------------|-------------------------------------|------------------------------------|
| 25 | Aluminum             | 7 to 9                              | 7.4 to 8.5                         |
|    | Nickel               | 12 to 16                            | 12.5 to 14                         |
|    | Cobalt               | 18 to 26                            | 21.5 to 24                         |
|    | Copper               | 2 to 4                              | 2.5 to 3.5                         |
|    | Carbon               | Below 0.1                           | Below 0.05                         |
|    | Manganese            | 0 to 1.0                            | Below 0.15                         |
| 30 | Silicon (Alnico V)   | 0.15 to 1.0                         | 0.4 to 0.7                         |
|    | Titanium (Alnico VI) | 0.2 to 2.0                          | 0.8 to 1.5                         |
|    | Columbium            | 0.05 to 1.0                         | 0.05 to 0.4                        |
|    | Sulphur              | 0.01 to 0.3                         | <sup>1</sup> 0.02 to 0.1           |

<sup>1</sup> At least  $\frac{1}{4}$  the amount of columbium.

35 Tests were made under conventional testing conditions of:

- (A)—A commercial Alnico V alloy containing zirconium and silicon.
- (B)—An Alnico V alloy containing silicon as its only additive.
- 40 (C)—A similar silicon-containing Alnico V alloy which also contained columbium and sulphur, in accordance with our invention.

45 (A)—The commercial zirconium- and silicon-containing Alnico V was selected for comparative purposes, as representative of the best available Alnico V alloy. Twenty-five heats of this alloy were used, having an average analysis as follows:

|    |           |                  |
|----|-----------|------------------|
| 50 | Aluminum  | 7.77%            |
|    | Nickel    | 13.40%           |
|    | Cobalt    | 22.70%           |
|    | Copper    | 2.83%            |
|    | Carbon    | Impurity, 0.026% |
| 55 | Manganese | Impurity, 0.08%  |
|    | Silicon   | 0.54%            |
|    | Zirconium | 0.26%            |
|    | Columbium | None             |
|    | Sulphur   | None             |

60 Tests of the twenty-five heats of this zirconium- and silicon-containing Alnico V alloy give results as shown in the following Table 2.

TABLE 2

Alnico V with zirconium and silicon

|               | Br     | He   | (BH)<br>max. |
|---------------|--------|------|--------------|
| High          | 13,550 | 664  | 5.76         |
| Low           | 12,120 | 600  | 5.15         |
| Average       | 12,800 | 630  | 5.50         |
| Percent Range | 11.8   | 11.3 | 11.8         |

In this Table 2, as in comparative tables given below, "Br" represents the residual magnetism per unit of the test piece after the test piece has been magnetized to its maximum value and the magnetizing force then reduced to zero; "Hc" represents the value of the demagnetizing force per unit of the test piece required to reduce the magnetization of the test piece from its Br value to zero; "(BH) max." is the maximum product, in millions, of B and H values at various points along the magnetization curve, and represents the amount of magnetic energy that each cubic centimeter of the test material is capable of supplying; the "high" values are the highest obtained with any test piece of the series; the "low" values are the lowest obtained with any test piece of the series; the "average" values are the average values of all the test pieces of the series; and "percent range" is the percentage of the range of values, i. e., the high value minus the low value, as compared to the low value.

B.—The Alnico V alloy containing silicon as its only additive was tested as a basis for comparison to show the effect of adding columbium and sulphur. Five heats of the silicon-containing Alnico V alloy were used. The same amounts and proportions of constituents were used in all five heats, and the five heats had the following average analysis:

|           | Percent |
|-----------|---------|
| Aluminum  | 7.63    |
| Nickel    | 13.14   |
| Cobalt    | 22.53   |
| Copper    | 2.76    |
| Carbon    | .028    |
| Manganese | .076    |
| Silicon   | .446    |

Tests of the five heats of this silicon-containing Alnico V alloy gave the results shown in the following Table 3.

TABLE 3  
Alnico V with silicon alone

|               | Br     | Hc  | (BH) max. |
|---------------|--------|-----|-----------|
| High          | 13,400 | 616 | 5.64      |
| Low           | 12,200 | 565 | 3.76      |
| Average       | 12,720 | 592 | 4.87      |
| Percent Range | 9.8    | 9.0 | 50        |

C.—The Alnico V alloy containing columbium and sulphur in accordance with the invention was prepared, treated, and tested in the same manner as the alloys described above. Eleven heats were used, as shown in the following Table 4. In such table, the first line shows in percentages the amounts of constituents, beside iron, which were charged to the furnace, and the following eleven lines show the percentages of constituents as found upon chemical analysis of the eleven different heats.

TABLE 4

| Heat No. | Al   | Ni    | Co    | Cu   | C    | Mn   | Si  | S    | Cb   |
|----------|------|-------|-------|------|------|------|-----|------|------|
| Charge   | 8    | 13.4  | 24    | 3    | .04  | .06  | .47 | .05  | .10  |
| 2009     | 7.86 | 13.52 | 23.21 | 3.06 | .04  | .08  | .49 | .031 | .10  |
| 2038     | 8.30 | 13.28 | 22.60 | 3.28 | .04  | .04  | .58 | .05  | .091 |
| 2051     | 7.82 | 13.52 | 23.04 | 3.22 | .03  | .03  | .53 | .033 | .098 |
| 2052     | 8.02 | 12.92 | 22.52 | 2.90 | .02  | .02  | .45 | .028 | .091 |
| 2053     | 8.02 | 13.34 | 22.88 | 3.18 | .02  | .03  | .51 | .032 | .076 |
| 2054     | 8.42 | 13.22 | 22.36 | 3.28 | .02  | .03  | .58 | .025 | .076 |
| 2055     | 7.94 | 12.86 | 22.60 | 3.24 | .02  | .03  | .60 | .027 | .084 |
| 2056     | 8.26 | 13.34 | 22.36 | 3.26 | .02  | .03  | .60 | .033 | .084 |
| 2364     | 7.46 | 13.82 | 23.54 | 3.18 | .02  | .01  | .47 | .043 | .086 |
| 2365     | 7.60 | 13.52 | 23.52 | 3.12 | .04  | .03  | .50 | .028 | .092 |
| 2442     | 7.90 | 13.76 | 23.36 | 3.12 | .03  | .02  | .51 | .05  | .081 |
| Average  | 7.96 | 13.37 | 22.91 | 3.17 | .027 | .032 | .53 | .034 | .087 |

<sup>1</sup> Represents amount charged, not analysis result.

Permeameter test bars were cast from these eleven columbium- and sulphur-containing Alnico V heats, were heat treated by standard Alnico V treatment, and were

then tested, and gave the magnetic data shown in the following Table 5.

TABLE 5

| Heat No. | Br     | Hc  | (BH) max. |
|----------|--------|-----|-----------|
| 2009     | 13,250 | 630 | 5.77      |
| 2038     | 13,450 | 623 | 5.84      |
| 2051     | 13,550 | 632 | 5.83      |
| 2052     | 13,450 | 644 | 5.87      |
| 2053     | 13,400 | 648 | 5.93      |
| 2054     | 13,300 | 636 | 5.80      |
| 2055     | 13,300 | 638 | 5.64      |
| 2056     | 13,200 | 645 | 5.75      |
| 2364     | 13,290 | 610 | 5.70      |
| 2365     | 13,380 | 624 | 5.71      |
| 2442     | 13,400 | 638 | 5.96      |

These results are summarized in the following Table 6:

TABLE 6

Alnico V with Si, S, and Cb.

|               | Br     | Hc  | (BH) max. |
|---------------|--------|-----|-----------|
| High          | 13,550 | 648 | 5.96      |
| Low           | 13,200 | 610 | 5.64      |
| Average       | 13,361 | 633 | 5.80      |
| Percent Range | 2.7    | 6.2 | 5.7       |

Samples of the eleven heats of the new alloy were tested for brittleness, and subjected to commercial working operations, and all were found to have good physical properties. All withstood the working operations, and none showed excess brittleness.

In comparison with Alnico V containing silicon alone (Table 3) the new columbium-containing Alnico V (Tables 5 and 6) is substantially improved. The "high" (BH) max. value was 5.96 as compared to 5.64, an improvement of 5.6%. The "low" (BH) max. value was 5.64 which was equal to the highest value obtained with the silicon-Alnico V. The average (BH) max. value was 5.80 as compared to 4.87, an improvement of nearly 20%. Moreover, the improved results were obtained uniformly, and the several heats of the new alloy were less subject to variation and gave substantially uniform high quality. Where the silicon-Alnico V heats varied over a range of 50% of the "low" value, the several heats of the new alloy varied only 5.7%. The addition of columbium, with sulphur, thus not only gave higher strength magnet metal, but gave improved uniformity as between successive heats.

The new columbium-containing Alnico V (tables 5 and 6) is also substantially improved over the zirconium-containing Alnico V alloy (Table 2) which represents the highest-strength material heretofore available. The "high" and "low" (BH) max. values of the new alloy are substantially higher than the corresponding values for the zirconium-containing alloy. The lowest value obtained with the new alloy was only about 2% below the highest value obtained with the zirconium-containing alloy. The new alloy gave an average (BH) max. value 5.5% higher than the zirconium-containing alloy. The new alloy gave much more uniform results, and the range of variation of results was less than half that obtained with the zirconium-containing alloy.

These improved results were obtained with a charge of only 0.10% of columbium, whereas the best available previous alloy contained 0.26% of zirconium, which is more expensive than the 0.10% of columbium. The new alloy was improved in magnetic properties, was obtained more uniformly, and was less in over all cost.

The improved Alnico V alloy, of the formula shown in Table 4, has been repeatedly made in regular commercial production, where a zirconium-containing Alnico V had previously been manufactured with the same facilities and under the same general conditions. It has been found

that the new columbium-containing alloy not only gives an improved product, but that the results of commercial manufacture are substantially more uniform than occurred with the zirconium-containing alloy. A similar comparative experience has been had with the Alnico VI alloy, and it has been found similarly that there was a substantial improvement in the uniformity of commercial production when the columbium-containing alloy was used instead of the zirconium-containing alloy.

We claim as our invention:

A permanent magnet consisting of an alloy containing from about 7.4% to about 8.5% aluminum, about 12.5% to about 14% nickel, about 21.5% to about 24% cobalt, about 2.5% to about 3.5% copper, about 0.4% to about 0.7% silicon, 0% to about 1.5% titanium, at 10

least 0.05% and not substantially more than approximately 0.1% columbium, an amount of sulphur at least equal to one-fourth the amount of columbium and not more than 0.1%, less than about 0.05% carbon, and less than about 0.15% manganese, the balance being substantially all iron.

References Cited in the file of this patent

UNITED STATES PATENTS

|           |          |       |               |
|-----------|----------|-------|---------------|
| 2,229,065 | Franks   | ----- | Jan. 21, 1941 |
| 2,395,285 | McKibben | ----- | Feb. 19, 1946 |
| 2,499,861 | Hansen   | ----- | Mar. 7, 1950  |
| 2,694,166 | Hadfield | ----- | Nov. 9, 1954  |